

**METHOD OF PRODUCING FIRE RESISTANT LIGNOCELLULOSE HARDBOARD PRODUCTS**

Walter P. Green, Jr., and Walter N. Meek, Jr., Laurel, Miss., assignors to Masonite Corporation, Laurel, Miss., a corporation of Delaware

No Drawing. Application April 13, 1955,  
Serial No. 501,194

7 Claims. (Cl. 117—103)

The present invention relates to the preparation of lignocellulose hardboard products characterized by greatly improved resistance to fire. More particularly, the invention relates to a novel method of impregnating hardboard sheets with water soluble phosphates in amounts sufficient to render the sheets fire retardant.

It has long been recognized by the hardboard, tileboard, and building industries that the production of fire retardant hardboard products would greatly enlarge their fields of usefulness. To this end, many proposals have been made to incorporate in hardboard products various fire proofing agents. It has been proposed, for example, to incorporate in these products such materials as borax, boric acid, nitrogen containing compounds, chlorinated hydrocarbons, and the like agents. The compounds have been added during the production of the hardboard and by impregnation of the finished product. However, the prior art methods have uniformly failed to accomplish the desired result. The treated hardboard has been subject to bleeding of the agents, crystallization thereof, and the like unsatisfactory properties. Above all, it has heretofore been almost impossible to obtain sufficient retention of the added agents to impart any great degree of fire resistance to the hardboard products.

We have now discovered, entirely unexpectedly, that water soluble phosphates may be incorporated into lignocellulose hardboard sheets in amounts which greatly improve the fire resistance of the products. In its generic aspect, therefore, the invention comprises the addition to lignocellulose hardboard sheets of water soluble ammonium phosphates in amounts sufficient to render the products fire retardant. More specifically, the invention is directed to impregnating hardboard products with a mixture of diammonium phosphate and monoammonium phosphate.

It has been found that lignocellulose hardboard sheets, having densities of about 1 or greater, may be first immersed in a hot concentrated aqueous solution of the phosphate mixture, and then immersed immediately in a cooler concentrated aqueous solution of the phosphate mixture whereby the sheets retain, upon drying and/or baking, from about 14% to about 20% of the phosphate salts based on the dry weight of the hardboard sheets. The treated sheets are characterized by greatly improved resistance to fire. The incorporated phosphate salts do not bleed out of the boards, and the products may be decorated with any desired coating agent such as air dried paint, baked enamel, decorative plastic sheets, and the treated boards may be laminated or glued by the use of selected adhesive materials.

The proportions of the two ammonium phosphates to be used are critical inasmuch as they tend to precipitate from the concentrated solutions employed in the novel method unless the limits established are closely adhered to. Broadly, the range of proportions suitable is from 2:1 to 1:2 parts by weight of diammonium phosphate to monoammonium phosphate. Within this operative range, it has been found that optimum results are obtained by

employing proportions of 1:1 to 1.25:1 parts by weight of diammonium phosphate to monoammonium phosphate.

The hot bath of concentrated aqueous phosphate mixture is preferably maintained at about 80% concentration although the amount of salts in solution will obviously vary somewhat as hardboard sheets are immersed therein. The boiling point of this concentrated solution is about 240° F. and it is preferable to maintain the bath at this temperature although the desired results are obtainable over a bath temperature range of about 230°—250° F.

The cooler second bath is preferably maintained at about 60% concentration of phosphate salts although the amount of salts in solution may vary by about 5% above or below the optimum concentration. It has been determined that the second bath should be maintained at about 120° F. plus or minus 20 degrees.

As stated before, the range of phosphate salts concentration and temperature ranges are critical inasmuch as the salts precipitate from solution where the stated limits are exceeded or fallen short of.

In carrying out the novel method of the invention, the selected hardboard sheet is first immersed in the hot bath for from about 3 minutes for the most dense sheet to about 1 minute in the case of a sheet of relatively low specific gravity such as about 1 or slightly less. Thereafter, the sheet is immediately immersed in the cooler bath for about 2—0.5 minute depending on the board density. Immersion times shorter than those specified result in insufficient phosphate salts content in the product. Immersion times greater than those specified are not desirable inasmuch as there is no necessity of exceeding 20% phosphate salts content in the product from the standpoint of fire resistance and, in addition, excessive amounts of salts in the sheet result in lowering the physical properties thereof. Upon removal of the sheet from the second bath, the solution remaining on the sheet surfaces may be removed as by washing with water and the impregnated sheet may be dried and/or baked. Uptake of phosphate salts lies within the range of about 14—20% based on the dry weight of the hardboard sheet.

Where the fire resistant sheet is to be coated with an air drying agent, it is only necessary to dry the sheet to remove water. However, where the impregnated sheet is to be finished with a baked enamel or similarly heat treated agent, it is preferable to bake the sheet to prevent gassing during curing of the enamel or other coating. It has been found that the baking cycle must be carried out over a progressively increasing temperature range of about 140°—275° F. extending over a period of about 12—16 hours. Subsequent to this baking treatment the sheet may be subjected to additional heat treatment without adversely affecting the coating material and without appreciable loss of fire resistance.

While the exact manner in which the hot-cold impregnation method functions is not known, it is believed that immersion of a hardboard in the hot bath serves to drive out some of the air and moisture present in the sheet. In this respect, it is important that the hardboard to be impregnated should have a minimum moisture content of 3.5% and preferably about 5%. Some impregnation of the hardboard occurs during this hot bath immersion. However, when the hot sheet is immersed in the second and relatively cool bath, there is apparently a vacuum effect on the voids present in the sheet. The cooler solution is thus enabled to penetrate the sheet very rapidly and thoroughly. In any event, much greater uptake of salts is obtained than by any single impregnation method. The result is the provision of hardboard containing sufficient ammonium phosphate salts to render the treated product fire retardant.

## 3

The invention will be more fully described by the following examples. It should be borne in mind, however, that the examples are given for illustrative purposes alone, and the invention is to be limited only by the scope of the appended claims.

5

## EXAMPLE 1

Several pieces of 49" square lignocellulose hardboard were prepared. The square hardboard sheets had specific gravities of about 1.12 and were smooth on both surfaces. In sequence, the boards were immersed in two aqueous solutions containing 1:1.25 proportions by weight of diammonium phosphate and monoammonium phosphate under the following conditions:

Solution 1—approximately 80% concentration of phosphate mixture. Temperature  $241^{\circ} \pm 1^{\circ}$  F. Boards immersed for 3 minutes.

Solution 2—approximately  $60 \pm 1.5\%$  concentration of phosphate mixture. Temperature  $122^{\circ} \pm 9^{\circ}$  F. Boards immersed for 2 minutes.

Escape of the evolved gases beneath the boards was permitted by use of a tilted hold-down for the boards. After being removed from the second solution, the boards were washed with water, allowed to drain, and dried employing a graduated temperature 16 hour baking cycle at  $140^{\circ}$ – $275^{\circ}$  F. The impregnated board products had an average specific gravity of 1.28 and contained an average of 18.3% of ammonium phosphate by weight. The treated boards were tested for flame resistance according to Federal Specification SS-A-118b of August 4, 1954, paragraphs 4.3.3, 4.3.3.1, 4.3.3.3 and 4.3.3.4. All results represent average figures for three tests:

## SS-A-118b Federal fire test (40 minute exposure)

|                  |                         |    |
|------------------|-------------------------|----|
| Weight loss      | 34.0%.                  | 35 |
| Initial flame    | 3 min. 28 sec.          | 35 |
| Cracked through  | 5 min. 20 sec.          | 35 |
| Pieces falling   | 8 min. 45 sec.          | 35 |
| Char diameter    | 27 inches.              | 35 |
| After flame time | None.                   | 40 |
| After glow time  | None.                   | 40 |
| After smoke      | 2.25 min. Light amount. | 45 |
| Rated            | Fire retardant.         | 50 |

In the above test, the sample is rated as fire retardant where the charred area does not extend to the edges of a 30 square inch area exposed to the flame employed.

In the following examples, the proportions of diammonium phosphate and monoammonium phosphate and impregnating times were varied over a wide range to illustrate the critical limits of the novel method of the invention.

## EXAMPLE 2

The procedure of Example 1 was repeated employing the following conditions:

Solution 1—approximately 80% concentration of phosphate mixture. Ratio—2 parts diammonium phosphate: 1 part monoammonium phosphate. Temperature  $255^{\circ}$  F. Board of specific gravity 1.04 immersed for 2.5 minutes.

Solution 2—approximately 58% concentration of phosphate mixture. Ratio of phosphates same as solution 1. Temperature  $127^{\circ}$  F. Board immersed for 1.5 minutes.

The impregnated board, after drying, had a phosphate salts content of 17.25% and a specific gravity of 1.17. The board was rated as fire retardant.

## EXAMPLE 3

The procedure of Example 1 was repeated employing the following conditions:

Solution 1—approximately 80% concentration of phosphate mixture. Ratio—2 parts diammonium phosphate: 1 part monoammonium phosphate. Temperature  $246^{\circ}$  F. Board of specific gravity 1.01 immersed for 1 minute.

Solution 2—approximately 54% concentration of phosphate mixture. Ratio of phosphates same as solution 1.

## 4

Temperature  $147^{\circ}$  F. Board immersed for 0.5 minute.

The impregnated board, after drying, had a phosphate salts content of 14.6% and a specific gravity of 1.17. The board was rated as fire retardant.

## EXAMPLE 4

The procedure of Example 1 was repeated employing the following conditions:

Solution 1—approximately 80% concentration of phosphate mixture. Ratio—1 part diammonium phosphate: 2 parts monoammonium phosphate. Temperature  $245^{\circ}$  F. Board of specific gravity 1.11 immersed for 3 minutes.

Solution 2—approximately 58% concentration of phosphate mixture. Ratio of phosphates same as solution 1. Temperature  $130^{\circ}$  F. Board immersed for 2 minutes.

The impregnated board, after drying, had a phosphate salts content of 17.1% and a specific gravity of 1.25. The board was rated as fire retardant.

All of the fire resistant products of the above examples were characterized by good appearance and physical properties equal to those of untreated hardboard. The products were coated with both air drying paint and baked enamels. The coated articles were entirely satisfactory in all respects.

From the foregoing description of the invention it will be seen that the novel method provides a desirable means for preparing fire resistant hardboard products. The invention has the outstanding advantage of providing a commercially acceptable method heretofore lacking in the prior art. The method is simple, economical, and provides fire resistant products which may be coated with any desired coating material either for general use or for use in the tileboard industry where perfection of the surface appearance is of prime importance.

We claim:

1. A method of imparting fire resistance to lignocellulose hardboard which comprises submerging a hardboard sheet in a hot aqueous solution of a mixture of diammonium phosphate and monoammonium phosphate for a period of time within the range of about 1–3 minutes, removing the hardboard sheet from the hot solution, immediately submerging the sheet in a cooler aqueous solution of a mixture of the said two phosphates for a period of time within the range of about 0.5–2 minutes, the two aqueous solutions containing parts by weight of the two phosphates within the range of 2:1 to 1:2 of diammonium phosphate to monoammonium phosphate, thereafter removing the excess solution from the surfaces of the hardboard sheet, and subjecting the impregnated sheet to a baking cycle.

2. A method of imparting fire resistance to lignocellulose hardboard which comprises submerging a hardboard sheet in a hot aqueous solution having a concentration of approximately 80% of a mixture of diammonium phosphate and monoammonium phosphate for a period of time within the range of about 1–3 minutes, removing the hardboard sheet from the hot solution, immediately submerging the sheet in a cooler aqueous solution containing a concentration of approximately 60% of the said two phosphates for a period of time within the range of about 0.5–2 minutes, the two aqueous solutions containing parts by weight of the two phosphates within the range of 2:1 to 1:2 of diammonium phosphate to monoammonium phosphate, thereafter removing the excess solution from the surfaces of the hardboard sheet, and subjecting the impregnated sheet to a baking cycle.

3. A method of imparting fire resistance to lignocellulose hardboard which comprises submerging a hardboard sheet in a hot aqueous solution having a concentration of approximately 80% of a mixture of diammonium phosphate and monoammonium phosphate for a period of time within the range of about 1–3 minutes, removing the hardboard sheet from the hot solution, immediately submerging the sheet in a cooler aqueous solution containing a concentration of approximately 60% of

the said two phosphates for a period of time within the range of about 0.5-2 minutes, the two aqueous solutions containing parts by weight of the two phosphates within the range of 2:1 to 1:2 of diammonium phosphate to monoammonium phosphate and the solutions being maintained at temperatures within the ranges of 230°-250° F. and 100°-140° F., respectively, thereafter removing the excess solution from the surfaces of the hardboard sheet, and subjecting the impregnated sheet to a baking cycle.

4. A method of imparting fire resistance to lignocellulose hardboard which comprises submerging a hardboard sheet in a hot aqueous solution having a concentration of approximately 80% of a mixture of diammonium phosphate and monoammonium phosphate for a period of time within the range of about 1-3 minutes, removing the hardboard sheet from the hot solution, immediately submerging the sheet in a cooler aqueous solution containing a concentration of approximately 60% of the said two phosphates for a period of time within the range of about 0.5-2 minutes, the two aqueous solutions containing parts by weight of the two phosphates within the range of 2:1 to 1:2 of diammonium phosphate to monoammonium phosphate and the solutions being maintained at temperatures within the ranges of 230°-250° F. and 100°-140° F., respectively, thereafter removing the excess solution from the surfaces of the hardboard sheet, and subjecting the impregnated sheet to a baking cycle at a graduated increasing temperature range of 140° F.-275° F. extending over a period of 12-16 hours.

5. A method of imparting fire resistance to lignocellulose hardboard which comprises submerging a hardboard sheet in a hot aqueous solution of a mixture of diammonium phosphate and monoammonium phosphate for a period of time within the range of about 1-3 minutes, removing the hardboard sheet from the hot solution, immediately submerging the sheet in a cooler aqueous solution of a mixture of the said two phosphates for a period of time within the range of about 0.5-2 minutes, the two aqueous solutions containing parts by weight of the two phosphates within the range of 1:1 to 1.25:1 of diammonium phosphate to monoammonium phosphate, thereafter removing the excess solution from the surfaces of the hardboard sheet, and subjecting the impregnated sheet to a baking cycle.

6. A method of impregnating a dense lignocellulose hardboard with from about 16% to about 20% by weight of water soluble phosphates which comprises submerging the hardboard sheet in a hot aqueous solution of a mixture of diammonium phosphate and monoammonium phosphate for about 3 minutes, removing the hardboard sheet from the hot solution, immediately submerging the sheet in a cooler aqueous solution of a mixture of the said two phosphates for about 2 minutes, the two aqueous solutions containing parts by weight of the two phosphates within the range of 1:1 to 1.25:1 of diammonium phosphate to monoammonium phosphate at concentrations of about 80% and 60% in the respective hot and cool solutions, thereafter removing the excess solution from the surfaces of the hardboard sheet, and drying the sheet.

7. A method of imparting fire resistance to lignocellulose hardboard which comprises submerging a hardboard sheet for about 3 minutes in an aqueous solution having a concentration of approximately 80% of a mixture containing equal parts by weight of diammonium phosphate and monoammonium phosphate, said solution being maintained at about 240° F., removing the hardboard sheet from the solution, immediately submerging the sheet in a second aqueous solution of said phosphates for about 2 minutes, said second solution containing similar 1:1 proportions of diammonium phosphate and monoammonium phosphate by weight at 60% concentration plus or minus about 5%, said second solution being maintained at about 120° F. plus or minus about 5° F., thereafter removing the excess solution from the surfaces of the hardboard sheet, and subjecting the impregnated sheet to a baking cycle at a graduated increasing temperature range of 140°-275° F. extending over a period of 12-16 hours.

References Cited in the file of this patent

UNITED STATES PATENTS

40 1,942,977 Payne ----- Jan. 9, 1934

FOREIGN PATENTS

1,126 Great Britain ----- 1875

1,187 Great Britain ----- 1856